



US007285516B2

(12) **United States Patent**  
**Carrick et al.**

(10) **Patent No.:** **US 7,285,516 B2**  
(45) **Date of Patent:** **Oct. 23, 2007**

(54) **ADDITIVE FORMULATION FOR  
LUBRICATING OILS**

(75) Inventors: **Virginia A. Carrick**, Chardon, OH (US); **William D. Abraham**, South Euclid, OH (US); **Gordon D. Lamb**, Southend Bradfield (GB); **R. Ian Wilby**, Wingerworth (GB); **James P Roski**, Wickliffe, OH (US)

(73) Assignee: **The Lubrizol Corporation**, Wickliffe, OH (US)

(\*) Notice: Subject to any disclaimer, the term of this patent is extended or adjusted under 35 U.S.C. 154(b) by 353 days.

(21) Appl. No.: **10/305,526**

(22) Filed: **Nov. 25, 2002**

(65) **Prior Publication Data**

US 2004/0102335 A1 May 27, 2004

(51) **Int. Cl.**

**C10M 141/08** (2006.01)

(52) **U.S. Cl.** ..... **508/192**; 508/372; 508/374; 508/390; 508/409; 508/414; 508/415; 508/479; 508/501; 508/502; 508/572; 508/585; 508/586

(58) **Field of Classification Search** ..... 508/192  
See application file for complete search history.

(56)

**References Cited**

U.S. PATENT DOCUMENTS

6,200,936 B1 3/2001 Moreton ..... 508/479  
6,310,009 B1 10/2001 Kocsis et al. ..... 508/186  
6,331,510 B1 \* 12/2001 Curtis et al. ..... 508/578  
6,340,659 B1 1/2002 Kocsis et al. ..... 508/518  
6,583,092 B1 \* 6/2003 Carrick et al. ..... 508/198  
6,846,782 B2 \* 1/2005 Calder ..... 508/293

FOREIGN PATENT DOCUMENTS

WO WO 01/56968 8/2001  
WO WO 02/062930 A 8/2002  
WO WO 03/104620 A 12/2003  
WO WO 2004/096957 A1 \* 11/2004

OTHER PUBLICATIONS

Mortier et al, "Chemistry and Technology of Lubricants," 2d ed 1997, pp. 77-82.

\* cited by examiner

*Primary Examiner*—Ellen M. McAvoy

(74) *Attorney, Agent, or Firm*—David M. Shold; Christopher D. Hilker

(57)

**ABSTRACT**

Lubricating oils containing an additive formulation including at least one sulphonate, saligenin and salixarate detergent provide improved wear performance and decreased sulphur and phosphorus emissions.

**17 Claims, No Drawings**

## 1

ADDITIVE FORMULATION FOR  
LUBRICATING OILS

## FIELD OF THE INVENTION

The present invention relates to the use of an additive formulation comprising in combination at least one sulphonate, saligenin, and salixarate detergent used in lubricating compositions. Optionally an additional detergent can be included. The use of saligenin and salixarate can allow reductions in the amount of overbased sulphonate detergent or sulphur-containing phenate detergent and zinc dialkyldithiophosphate, especially in diesel engines.

## BACKGROUND OF THE INVENTION

It is well known for lubricating oils to contain a number of additives used to protect the engine from wear, soot deposits and acidity build up. Common additives for engine lubricating oils include zinc dialkyldithiophosphate (ZDDP) an antiwear additive, and overbased calcium sulphonate and calcium phenate detergents. It is believed that ZDDP anti-wear additives protect the engine by forming a protective film on metal surfaces. Detergents such as overbased calcium sulphonate help keep the engine parts clean of soot and other deposits, and offer an alkalinity reserve. Typical treatment quantities of ZDDP range from 1 to 2 weight percent based on the total weight of the lubricant. Typical treatment quantities of overbased calcium sulphonate range from 0.05 to 5 weight percent based on the total weight of the lubricant.

In recent years phosphorus compounds and sulphur (from sulphonates, sulphur-containing phenates, and other materials such as metal-containing dithiophosphates) derived from engine lubricants have been shown to contribute in part to particulate emissions. Also, sulphur and phosphorus tend to poison the catalysts used in catalytic converters, resulting in a reduction in performance of said catalysts.

However, any reduction in the amount of ZDDP or overbased calcium sulphonates or phenates will reduce the antiwear, detergent, and reserve alkalinity properties of the lubricant. Therefore there is a need for an additive package that will reduce sulphur and phosphorus content without having an adverse effect on these properties of lubricant oil.

U.S. Pat. No. 6,310,009, Kocsis et al., Oct. 30, 2001, relates to the use of saligenin derivatives used in lubricating compositions. The formulations contain borated or non-borated magnesium saligenin derivatives. These compositions exhibit improved seal compatibility and reduced copper and lead corrosion.

U.S. Pat. No. 6,200,936, Moreton, Mar. 13, 2001, relates to the use of salixarate compounds as an additive for finished lubricating oils. The compositions disclosed are particularly suitable for medium or low speed diesel engines, especially four-stroke trunk piston engines.

PCT publication WO 01/56968, Aug. 9, 2001, relates to the use of salixarate type compounds used in lubricating oils. The compositions disclosed are particularly suitable as thermal stabilisers for medium or low speed diesel engines.

The present invention provides an additive formulation for lubricating oils capable of decreasing sulphur and phosphorus containing emissions. It further can lead to decreased engine wear and decreased corrosion. The invention further provides an additive formulation for lubricating oils with low phosphorus and sulphur content capable of meeting or exceeding current requirements of engine cleanliness, wear protection, and alkalinity. It further provides an additive

## 2

formulation for lubricating oils capable of producing reduced amounts of ash and capable of improving seal compatibility.

## SUMMARY OF THE INVENTION

The present invention provides a composition comprising:

- a. a mono- or divalent metal sulphonate detergent;
  - b. a mono- or divalent metal salixarate detergent;
  - c. a mono- or divalent metal saligenin detergent; and
  - d. optionally an additional mono- or divalent metal detergent other than (a), (b) or (c); and,
- an oil of lubricating viscosity.

In one embodiment, the mono- or divalent metal can comprise calcium, magnesium, lithium, potassium or sodium.

It further provides a lubricant composition comprising a major amount of oil of lubricating viscosity and a minor amount of at least one of each of the following:

- a. a detergent,
- b. a dispersant,
- c. an antiwear agent, and
- d. an antioxidant;

characterised in that the detergent comprises in combination at least one mono- or divalent metal sulphonate detergent, at least one mono- or divalent metal salixarate detergent, and at least one mono- or divalent metal saligenin detergent, and optionally an additional mono- or divalent metal detergent other than the foregoing.

The invention further provides a method for lubricating an internal combustion engine, comprising supplying thereto a lubricant comprising the composition as described herein.

The use of a combination of a metal sulphonate, metal salixarate, and metal saligenin allows a reduction in the amount of metal sulphonate detergents and metal dialkyldithiophosphates and related antiwear additives levels in the lubricating oil composition. This reduction in phosphorus and sulphur containing additives allows the development of a formulation that meets current lubricating oil requirements with a lubricant having low phosphorus and sulphur content.

DETAILED DESCRIPTION OF THE  
INVENTION

Hereinafter the saligenin detergent, salixarate detergent, and sulphonate detergent are referred to as saligenin, salixarate and sulphonate. Unless otherwise stated all weight percents are based on the amount of finished lubricant.

It has been found, that an additive formulation used in a lubricating composition, comprising an oil of lubricating viscosity, in combination at least one detergent mono- or divalent metal sulphonate, at least one detergent mono- or divalent metal salixarate and at least one detergent mono- or divalent metal saligenin produces reduced amounts of sulphur, phosphorus, ash, engine wear and corrosion. The additive formulation is described as follows:

## Additive Composition

Generally, the composition of the present invention comprises:

- a. a mono- or divalent metal sulphonate in an amount 0.05 to 1.5 weight percent;
- b. a mono- or divalent metal salixarate in an amount 0.1 to 5 weight percent;

- c. a mono- or divalent metal saligenin in an amount 0.1 to 4.2 weight percent and
- d. an oil of lubricating viscosity in an amount up to 99.75 weight percent

Often the additive formulation in oil with a lubricating viscosity lubricant composition comprises said sulphonate in an amount 0.1 to 1.2 weight percent. More preferably said sulphonate is present in an amount 0.15 to 0.8 weight percent.

Often the additive formulation in oil with a lubricating viscosity lubricant composition comprises said salixarate in an amount 0.15 to 3 weight percent. More preferably said salixarate is present in an amount 0.2 to 2 weight percent.

Often the additive formulation in oil with a lubricating viscosity comprises said saligenin in an amount 0.15 to 3 weight percent. More preferably said saligenin is present in an amount 0.2 to 1.7 weight percent.

If the present invention is in the form of a concentrate (which can be combined with additional oil to form, in whole or in part, a finished lubricant), the amount of each of the above-mentioned detergents, as well as the other components, will be present in a concentration which is approximately 5 or 10-fold greater than the values given above. The amount of oil will be correspondingly reduced.

Often the additive formulation in oil with a lubricating viscosity, i.e., as a fully formulated lubricant composition, has a total sulphur content below 0.5 weight percent. More preferably, the total sulphur content is below 0.3 weight percent.

Often the additive formulation in oil with a lubricating viscosity, i.e., as a fully formulated lubricant composition, has a total phosphorus content below 0.1 weight percent. More preferably, the total phosphorus content is below 0.085 or even 0.06, 0.055, or 0.05 weight percent or lower. It is noted that a common source of phosphorus in engine lubricants is zinc dialkyl dithiophosphate (ZDDP), a very commonly used anti-wear agent. The present invention encompasses formulations which contain ZDDP at an appropriate level.

Often the additive formulation in oil with a lubricating viscosity, i.e., as a fully formulated lubricant composition, has a total sulphated ash content below 1.5 weight percent. More preferably the sulphated ash content is below 1.1 weight percent or even 1.0, 0.8 or 0.5 weight percent.

#### Saligenin Derivative

The saligenin component of the additive formulation can be represented by the formula:



wherein X comprises  $-\text{CHO}$  or  $-\text{CH}_2\text{OH}$ , Y comprises  $-\text{CH}_2-$  or  $-\text{CH}_2\text{OCH}_2-$ , and wherein such  $-\text{CHO}$  groups comprise at least 10 mole percent of the X and Y groups; M is a mono- or di-va lent metal ion. Each n is independently 0 or 1.  $\text{R}^1$  is a hydrocarbyl group containing 1 to 60 carbon atoms, m is 0 to 10, and when  $m > 0$ , one of

the X groups can be H; each p is independently 0, 1, 2 or 3, preferably 1; and that the total number of carbon atoms in all  $\text{R}^1$  groups is at least 7.

When n is 0, M is replaced by H to form an unneutralised phenolic  $-\text{OH}$  group. The average number of unneutralised phenolic groups can be between 0 and 100 percent. This results in the compound being partially or wholly neutralised with one or more monovalent or divalent metal ions.

Preferred metal ions M are monovalent metals ion such as 10 lithium, sodium, potassium. The monovalent metal ions can be used alone or in combination with hydrogen, ammonium or divalent metal ions.

More preferably M is a divalent metal ion such calcium or magnesium. The divalent metal ions can be used alone or in 15 combination with hydrogen, ammonium or monovalent metal ions. Most preferably the metal ion is magnesium.

The number of magnesium ions in the composition is typically 10-100% of the amount required for complete neutralisation, or, in another embodiment, 40-90%, or alternatively 60-80% neutralisation by magnesium. Since magnesium is normally a divalent ion, it can neutralise up to two phenolic hydroxy groups. The two hydroxy groups may be on the same or on different molecules. If the value of n is less than 1.0, this indicates that the hydroxy groups are less than 25 completely neutralised by magnesium ions. Alternatively, each magnesium ion can be associated with one phenolic anion and an ion of another type such as a hydroxide ion or carbonate ion ( $\text{CO}_3^{2-}$ ), while still providing an n value of 1.0.

30 The specification that the average value of n is 0.1 to 1.0 is not directly applicable to overbased versions of this material (described below and also a part of the present invention) in which an excess of Mg or another cation can be present. It should be understood that, even in an overbased material, some fraction of the phenolic OH groups may not have reacted with the magnesium and may retain the OH structure.

Most of the rings contain at least one  $\text{R}^1$  substituent, which is a hydrocarbyl group, preferably an alkyl group, 40 containing 1 to 60 carbon atoms, preferably 7 to 28 carbon atoms, more preferably 9 to 18 carbon atoms. It is understood that  $\text{R}^1$  will normally comprise a mixture of various chain lengths, so that the foregoing numbers will normally represent an average number of carbon atoms in the  $\text{R}^1$  groups (number average).  $\text{R}^1$  can be linear or branched. Each ring in the structure will be substituted with 0, 1, 2, or 3 such  $\text{R}^1$  groups (that is, p=0, 1, 2, or 3), most typically 1, although different rings in a given molecule may contain different numbers of such substituents. At least one aromatic ring in 45 the molecule must contain at least one  $\text{R}^1$  group, and the total number of carbon atoms in all the  $\text{R}^1$  groups in the molecule segment should be at least 7, preferably at least 12.

In the above structure the X and Y groups may be seen as 50 groups derived from formaldehyde or a formaldehyde source, by condensative reaction with the aromatic molecule. While various species of X and Y may be present in the molecules in question, the commonest species comprising X are  $-\text{CHO}$  (aldehyde functionality) and  $-\text{CH}_2\text{OH}$  (hydroxymethyl functionality); similarly the commonest 55 species comprising Y are  $-\text{CH}_2-$  (methylene bridge) and  $-\text{CH}_2\text{OCH}_2-$  (ether bridge).

In one embodiment, X is at least in part  $-\text{CHO}$ , and such 60  $-\text{CHO}$  groups comprise at least 10, 12, or 15 mole percent of the X and Y groups. Preferably the  $-\text{CHO}$  groups comprise 20 to 60 mole percent of the X and Y groups and more preferably 25 to 40 mole percent of the X and Y groups.

In another embodiment, X is at least in part  $-\text{CH}_2\text{OH}$  and such  $-\text{CH}_2\text{OH}$  groups comprise 10 to 50 mole percent of the X and Y groups, preferably 15 to 30 mole percent of the X and Y groups.

In an embodiment in which m is non-zero, Y is at least in part  $-\text{CH}_2-$ , and such  $-\text{CH}_2-$  groups comprise 25 to 55 mole percent of the X and Y groups, preferably 32 to 45 mole percent of the X and Y groups.

In another embodiment Y is at least in part  $-\text{CH}_2\text{OCH}_2-$ , and such  $-\text{CH}_2\text{OCH}_2-$  groups comprise 5 to 20 mole percent of the X and Y groups, and preferably 10 to 16 mole percent of the X and Y groups.

The relative amounts of the various X and Y groups depends to a certain extent on the conditions of synthesis of the molecules. Under many conditions the amount of  $-\text{CH}_2\text{OCH}_2-$  groups is relatively small compared to the other groups and is reasonably constant at 13 to 17 mole percent. Ignoring the amount of such ether groups and focusing on the relative amounts of the  $-\text{CHO}$ ,  $-\text{CH}_2\text{OH}$ , and  $-\text{CH}_2-$  groups, it has been found that particularly preferred compositions have the following relative amounts of these three groups, the total of such amounts in each case being normalized to equal 100%:

$-\text{CHO}$ : 15-100%, preferably 20-80%, more preferably 25-40%  
 $-\text{CH}_2\text{OH}$ : 0-54%, preferably 2-46%, more preferably 10-40%  
 $-\text{CH}_2-$ : 0-64%, preferably 18-64%, more preferably 20-60%

Saligenin derivatives and methods of their preparation are described in greater detail in U.S. Pat. No. 6,310,009.

As used herein, the term "hydrocarbyl substituent" or "hydrocarbyl group" is used in its ordinary sense, which is well-known to those skilled in the art. Specifically, it refers to a group having a carbon atom directly attached to the remainder of the molecule and having predominantly hydrocarbon character.

Examples of hydrocarbyl groups include:

- (1) hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form a ring);
- (2) substituted hydrocarbon substituents, that is, substituents containing non-hydrocarbon groups which, in the context of this invention, do not alter the predominantly hydrocarbon substituent (e.g., halo (especially chloro and fluoro), hydroxy, alkoxy, mercapto, alkylmercapto, nitro, nitroso, and sulfoxo);
- (3) hetero substituents, that is, substituents which, while having a predominantly hydrocarbon character, in the context of this invention, contain other than carbon in a ring or chain otherwise composed of carbon atoms. Heteroatoms include sulfur, oxygen, nitrogen, and encompass substituents as pyridyl, furyl, thieryl and imidazolyl. In general, no more than two, preferably no more than one, non-hydrocarbon substituent will be present for every ten carbon atoms in the hydrocarbyl group; typically, there will be no non-hydrocarbon substituents in the hydrocarbyl group.

#### Salixarate Derivative

The salixarate component of the additive formulation can be represented by a substantially linear compound comprising at least one unit of formula (I) or formula (II):



each end of the compound having a terminal group of formula (III) or formula (IV):



such groups being linked by divalent bridging groups A, which may be the same or different for each linkage; wherein in formulas (I)-(IV) R³ is hydrogen or a hydrocarbyl group; R² is hydroxyl or a hydrocarbyl group and j is 0, 1, or 2; R⁶ is hydrogen, a hydrocarbyl group, or a hetero-substituted hydrocarbyl group; either R⁴ is hydroxyl and R⁵ and R⁷ are independently either hydrogen, a hydrocarbyl group, or hetero-substituted hydrocarbyl group, or else R⁵ and R⁷ are both hydroxyl and R⁴ is hydrogen, a hydrocarbyl group, or a hetero-substituted hydrocarbyl group; provided that at least one of R⁴, R⁵, R⁶ and R⁷ is hydrocarbyl containing at least 8 carbon atoms; and wherein the molecules on average contain at least one of unit (I) or (III) and at least one of unit (II) or (IV) and the ratio of the total number of units (I) and (III) to the total number of units of (II) and (IV) in the composition is about 0.1:1 to about 2:1.

The divalent bridging group "A," which may be the same or different in each occurrence, includes  $-\text{CH}_2-$  (methylene bridge) and  $-\text{CH}_2\text{OCH}_2-$  (ether bridge), either of which may be derived from formaldehyde or a formaldehyde equivalent (e.g., paraform, formalin).

Salixarate derivatives and methods of their preparation are described in greater detail in U.S. Pat. No. 6,200,936 and PCT Publication WO 01/56968. It is believed that the salixarate derivatives have a predominantly linear, rather

than macrocyclic, structure, although both structures are intended to be encompassed by the term "salixarate."

Preparative Example A. Overbased Salixarate

Step (a). A reactor is charged with 15 kg (23.3 moles) of polyisobuteneyl ( $M_n$  550) substituted phenol and 10.7 kg 150 N mineral oil. The materials are heated, under nitrogen, to 35° C., then 120 g (1.07 moles) aqueous KOH is added along with 100 mL distilled water wash. The mixture is heated to 75° C. over 0.5 hour and 2.6 kg (32.1 moles) of 37% aqueous formaldehyde is added over 0.5 hour along with 300 mL distilled water wash. The mixture is held at temperature for 2 hours, whereupon 1.65 kg salicylic acid (12 moles) is added followed by heating to 99° C. and reflux. The reaction mixture is further heated to 140° C. over 1 hour, removing 2.6 L aqueous distillate. The mixture is maintained at 140° C. for 1.5 hour at atmospheric pressure, followed by reduced pressure, collecting some additional aqueous distillate.

Step (b). A reactor is charged with 13.0 kg (8.95 moles) of the cooled product of step (a), 2.33 kg (31.5 moles)  $Ca(OH)_2$ , and 450 g ethylene glycol. While stirring, 7.38 kg of 2-ethylhexanol are added over 0.3 hours. The mixture is heated at 95° C. at reduced pressure over 3/4 hour, followed by 130° C. over 1/4 hour, during which time 0.5 L aqueous distillate is collected. An additional 2.16 kg ethylene glycol is added is added over about 0.3 hour at 125 to 130° C. Carbon dioxide is passed into the mixture under slight vacuum at 500 g/hour until a total of 750 g is added. After carbonation is complete, the temperature is increased to 200° C. and maintained for a total of about 2.2 hours, during which time 9.5 L aqueous distillate is collected. The product is an overbased calcium salixarate.

It is believed that a significant fraction of salixarate molecules (prior to neutralisation) may be represented on average by the following structure:



where each R is an alkyl group, and, in a preferred embodiment, is a polyisobutene group (especially of molecular weight 200-1,000, or about 550). Significant amounts of di- or trinuclear species may also be present containing one salicylic end group (III).

Sulphonate Derivative

The sulphonate component of the additive formulation can be represented by the formula:



wherein,  $R^8$  is independently alkyl, cycloalkyl, aryl, acyl, or hydrocarbyl groups with a 6 to 30 carbon atoms, and M is a metal ion. k is independently 1, 2, 3, or 4.

Preferred monovalent metal ions M include lithium, sodium, and potassium. The monovalent metal ions can be used alone or in combination with ammonium or divalent metal ions.

More preferably M is a divalent metal ion such calcium or magnesium. The divalent metal ions can be used alone or in combination with hydrogen, ammonium or monovalent metal ions. Most preferably the metal ion is calcium.

In one embodiment, k is 1 or 2 and  $R^8$  is a branched or linear alkyl substituent with 6 to 40 carbons. More preferably, the alkyl substituent comprises 8 to 25 carbons. Even more preferably the alkyl substituent comprises 10 to 20 carbons. The most preferred sulphonate components are calcium polypropene benzenesulfonate and calcium mono and dialkyl ( $C>10$ ) benzenesulfonate. Sulphonate derivatives and methods of their preparation are described in greater detail in "Chemistry and Technology of Lubricants", 2<sup>nd</sup> Edition, Edited by R. M. Mortier and S. T. Orszulik 1997.

Overbased Salts

Each of the sulfonate, saligenin, and salixarate can be overbased detergents. Overbased materials, otherwise referred to as overbased or superbased salts, are generally single phase, homogeneous Newtonian systems characterized by a metal content in excess of that which would be present for neutralization according to the stoichiometry of the metal and the particular acidic organic compound reacted with the metal. The overbased materials are prepared by reacting an acidic material (typically an inorganic acid or lower carboxylic acid, preferably carbon dioxide) with a mixture comprising an acidic organic compound, a reaction medium comprising at least one inert, organic solvent (mineral oil, naphtha, toluene, xylene, etc.) for said acidic

organic material, a stoichiometric excess of a metal base, and a promoter such as a phenol or alcohol. The acidic organic material will normally have a sufficient number of carbon atoms to provide a degree of solubility in oil. The amount of excess metal is commonly expressed in terms of metal ratio. The term "metal ratio" is the ratio of the total equivalents of the metal to the equivalents of the acidic organic compound. A neutral metal salt has a metal ratio of one. A salt having 4.5 times as much metal as present in a normal salt will have metal excess of 3.5 equivalents, or a ratio of 4.5.

Such overbased materials are well known to those skilled in the art. Patents describing techniques for making basic salts of sulphonic acids, carboxylic acids, phenols, phosphonic acids, and mixtures of any two or more of these include U.S. Pat. Nos. 2,501,731; 2,616,905; 2,616,911; 2,616,925; 2,777,874; 3,256,186; 3,384,585; 3,365,396; 3,320,162; 3,318,809; 3,488,284; and 3,629,109.

## The Optional Additional Detergent

If desired, an additional detergent may be present beside those described above. In one instance, it is understood that commercially available detergents of the sulphonate, salixarate, or saligenin type may be prepared in the presence of a small amount of another detergent. In other embodiments, the additional detergent or detergents may be separately added as additional components. Among the types of additional detergents that can be included are carboxylate detergents, and phenol-based detergents. Both the aforementioned salixarate detergent and the saligenin detergent may also be considered phenol based detergents in that they will contain phenolic functionality. For this reason the additional detergent, for clarity, is designated as being distinct from the salixarate or saligenin detergent. The phenol-based detergent can be a hydrocarbyl-substituted phenate detergent, a sulphurised hydrocarbyl-substituted phenate detergent, a formaldehyde linked hydrocarbyl-substituted phenate detergent, or a hydrocarbyl-substituted salicylate detergent. Salicylates are also carboxy-containing materials, but they will be generally considered herein as a species of a phenol-based detergent. The additional detergent will typically be overbased, as described above and using the general methods described above.

Carboxylic detergents are typically metal overbased carboxylic acids having a sufficiently long hydrocarbon moiety to promote oil solubility. They are well known commercial materials and can be prepared by known methods from aliphatic, cycloaliphatic, and aromatic mono- and polybasic carboxylic acids. They generally contain at least 8 carbon atom, preferably at least 12 carbon atoms, and typically up to 400 carbon atoms. Examples include 2-ethylhexanoic acid, linoleic acid, propylene-tetramer-substituted maleic acid, isostearic acid, oleic acid, dioctylcyclopentanecarboxylic acid, and mixtures of acids such as tall oil acids and rosin acids. A more detailed listing and description of suitable carboxylic acids, and a list of references describing methods for preparing overbased salts thereof, is found in U.S. Pat. No. 5,824,626, columns 9-11.

Phenate detergents are typically metal overbased phenols having a sufficiently long hydrocarbon substituent to promote oil solubility. The phenols from which the phenates are formed are of the general formula  $R_n(AR)-(XH)_m$ . In this formula, R is an aliphatic hydrocarbon based (hydrocarbyl) group of at least 4 carbon atoms, and normally no more than 400 carbon atoms, n is an integer of 1 to 4, AR is a polyvalent aromatic hydrocarbon nucleus of up to 14 carbon atoms (preferably a benzene nucleus), each X is independently sulphur or oxygen, preferably oxygen, and m is an integer of 1 to 4. Preferably there is an average of at least 8 aliphatic carbon atoms provided by the R groups for each phenol molecule. Examples included hexylphenol, cyclohexylphenol, heptylphenol, nonylphenol, dodecylphenol, and other hydrocarbon-substituted phenols. Phenols and their conversion into phenate detergents described in greater detail in U.S. Pat. No. 5,824,626 (columns 11 and 12) and U.S. Pat. No. 3,372,116.

Other phenates that are useful are those that are made from phenols that have been linked through alkylene (e.g., methylene) bridges. These are made by reacting single or multi-ring phenols with aldehydes or ketones, typically in the presence of an acid or basic catalyst.

Sulphurised phenate detergents are prepared from phenols which have been sulphurised by reacting with a sulphurising agent such as sulphur, a sulphur halide, or sulphide or hydrosulphide salt, typically by mixing at a temperature above 60° C., depending on the reactivity of the sulphurising

agent. The products include sulphides, polysulphides, and other products from such reaction. The molar ratio of the phenol to the sulphur compound can be from 1:0.5 to 1:1.5 or even higher. Synthesis of sulphurised phenate detergents is described in greater detail in U.S. Pat. No. 2,680,096 and U.S. Pat. No. 3,372,116, including columns 2 and 3.

Salicylate detergents can be considered a species of phenate detergent, since salicylic acid contains a phenolic OH group. They may also be considered a species of carboxylic acid, since salicylic acid contains a carboxy group, COOH. Typical salicylate detergents are metal overbased salicylates having a sufficiently long hydrocarbon substituent to promote oil solubility. Hydrocarbyl-substituted salicylic acids can be prepared by the reaction of the corresponding phenol by reaction of an alkali metal salt thereof with carbon dioxide. The hydrocarbon substituent can be as described for the carboxylate or phenate detergents. Overbased salicylic acid detergents and their preparation are described in greater detail in U.S. Pat. No. 3,372,116.

A preferred amount of the optional detergent is typically 0.1 to 2 percent by weight, or 0.12 to 1.2 percent, or 0.3 to 0.8 percent.

## 25 Oil of Lubricating Viscosity

The lubricating compositions and functional fluids of the present invention are based on diverse oils of lubricating viscosity, including natural and synthetic lubricating oils and mixtures thereof. Synthetic oils may be produced by Fischer-Tropsch reactions.

The lubricant compositions of this invention employ an oil of lubricating viscosity which is generally present in a major amount (i.e. an amount greater than 50% by weight). Generally, the oil of lubricating viscosity is present in an amount greater than 60%, or greater than about 70%, or greater than 80% by weight of the composition. In a concentrate, the amount of oil is correspondingly reduced.

Natural oils useful in making the inventive lubricants and functional fluids include animal oils and vegetable oils (e.g., castor oil, lard oil) as well as mineral lubricating oils such as liquid petroleum oils and solvent-treated or acid-treated mineral lubricating oils of the paraffinic, naphthenic or mixed paraffinic-naphthenic types. Oils of lubricating viscosity derived from coal or shale are also useful. Synthetic lubricating oils are useful and include hydrocarbon oils such as polymerised and interpolymerised olefins (e.g., polybutylenes, polypropylenes, propyleneisobutylene copolymers,); poly(1-hexenes), poly(1-octenes), poly(1-decenes), and mixtures thereof; alkyl-benzenes (e.g., dodecylbenzenes, tetradecylbenzenes, dinonylbenzenes, di-(2-ethylhexyl)-benzenes,); polyphenyls (e.g., biphenyls, terphenyls, alkylated polyphenyls,); alkylated diphenyl ethers and alkylated diphenyl sulfides and the derivatives, analogs and homologs thereof.

Alkylene oxide polymers and interpolymers and derivatives thereof where the terminal hydroxyl groups have been modified by esterification, and etherification, constitute another class of known synthetic lubricating oils that can be used. These are exemplified by the oils prepared through polymerisation of ethylene oxide or propylene oxide, the alkyl and aryl ethers of these polyoxyalkylene polymers (e.g., methyl-polyisopropylene glycol ether having a number average molecular weight of 1000, diphenyl ether of polyethylene glycol having a molecular weight of 500-1000, diethyl ether of polypropylene glycol having a molecular weight of 1000-1500) or mono- and polycarboxylic esters

thereof, for example, the acetic acid esters, mixed C<sub>3-8</sub> fatty acid esters, or the C<sub>13</sub> Oxo acid diester of tetraethylene glycol.

Another suitable class of synthetic lubricating oils that can be used comprises the esters of dicarboxylic acids (e.g., phthalic acid, succinic acid, alkyl succinic acids, alkenyl succinic acids, maleic acid, azelaic acid, suberic acid, sebacic acid, fumaric acid, adipic acid, linoleic acid dimer, malonic acid, alkyl malonic acids, and alkenyl malonic acids) with a variety of alcohols (e.g., butyl alcohol, hexyl alcohol, dodecyl alcohol, 2-ethylhexyl alcohol, ethylene glycol, diethylene glycol monoether, and propylene glycol). Specific examples of these esters include dibutyl adipate, di-(2-ethylhexyl) sebacate, di-n-hexyl fumarate, dioctyl sebacate, diisooctyl azelate, diisodecyl azelate, dioctyl phthalate, didecyl phthalate, dieicosyl sebacate, the 2-ethylhexyl diester of linoleic acid dimer, and the complex ester formed by reacting one mole of sebacic acid with two moles of tetraethylene glycol and two moles of 2-ethylhexanoic acid.

Esters useful as synthetic oils also include those made from C<sub>5</sub> to C<sub>12</sub> monocarboxylic acids and polyols and polyol ethers such as neopentyl glycol, trimethylol propane, pentaerythritol, dipentaerythritol, and tripentaerythritol.

Silicon-based oils such as the polyalkyl-, polyaryl-, polyalkoxy-, or polyaryloxy-siloxane oils and silicate oils comprise another useful class of synthetic lubricants (e.g., tetraethyl silicate, tetraisopropyl silicate, tetra-(2-ethylhexyl) silicate, tetra-(4-methylhexyl)silicate, tetra-(p-tert-butylphenyl) silicate, hexyl-(4-methyl-2-pentoxy) disiloxane, poly(methyl) siloxanes, and poly-(methylphenyl)siloxanes). Other synthetic lubricating oils include liquid esters of phosphorus-containing acids (e.g., tricresyl phosphate, trioctyl phosphate, and the diethyl ester of decane phosphonic acid), and polymeric tetrahydrofurans.

Unrefined, refined and re-refined oils, either natural or synthetic (as well as mixtures of two or more of any of these) of the type disclosed hereinabove can be used in the lubricants of the present invention. Unrefined oils are those obtained directly from a natural or synthetic source without further purification treatment. For example, a shale oil obtained directly from retorting operations, a petroleum oil obtained directly from primary distillation or ester oil obtained directly from an esterification process and used without further treatment would be an unrefined oil. Refined oils are similar to the unrefined oils except they have been further treated in one or more purification steps to improve one or more properties. Many such purification techniques are known to those skilled in the art such as solvent extraction, secondary distillation, acid or base extraction, filtration, percolation, Re-refined oils are obtained by processes similar to those used to obtain refined oils applied to refined oils which have been already used in service. Such re-refined oils are also known as reclaimed or reprocessed oils and often are additionally processed by techniques directed to removal of spent additives and oil breakdown products.

Oils of lubricating viscosity can also be defined as specified in the American Petroleum Institute (API) Base Oil Interchangeability Guidelines. The five base oil groups are as follows:

| Base Oil Category | Sulphur (%)                                         | and/or | Saturates (%) | Viscosity Index |
|-------------------|-----------------------------------------------------|--------|---------------|-----------------|
| Group I           | >0.03                                               |        | <90           | 80-120          |
| Group II          | ≤0.03                                               | and    | ≥90           | 80-120          |
| Group III         | ≤0.03                                               | and    | ≥90           | ≥120            |
| Group IV          | All polyalphaolefins (PAOs)                         |        |               |                 |
| Group V           | All others not included in Groups I, II, III, or IV |        |               |                 |

10

Groups I, II, and III are mineral oil base stocks. In one embodiment, the oil of lubricating viscosity in the present invention comprises a Group II, III, IV, or V oil or mixtures thereof. That is, a major portion of the oil can be of group II through V, optionally mixed with a minor portion of Group I oil.

#### The Antioxidant

In a further embodiment, the lubricating oil composition may also contain an antioxidant. Antioxidants for use in lubricant compositions are well known and include a variety of chemical types including phenate sulfides, phosphosulphurised terpenes, sulphurised esters, aromatic amines, and hindered phenols.

A preferred antioxidant is a sterically hindered phenol. Such antioxidants are typically alkyl phenols of the formula:



wherein R<sup>9</sup> and R<sup>10</sup> are independently branched or linear alkyl groups containing 1 up to 24 carbon atoms. Preferably R<sup>9</sup> and R<sup>10</sup> contain 4 to 18 carbon atoms and most preferably from 4 to 12 carbon atoms. R<sup>9</sup> and R<sup>10</sup> may be either straight chained or branched chained; branched chained is generally preferred. Preferably the phenol is a butyl substituted phenol containing two t-butyl groups. When the t-butyl groups occupy the 2,6-position, that is, the phenol is sterically hindered. J is H, hydrocarbyl, or a bridging group between two such aromatic groups. Bridging groups in the para position (J) include —CH<sub>2</sub>— (methylene bridge) and —CH<sub>2</sub>OCH<sub>2</sub>— (ether bridge).

A particularly preferred antioxidant is a hindered, ester-substituted phenol such as one represented by the formula:



wherein R<sup>11</sup> is a straight chain or branched chain alkyl group containing 2 to 22 carbon atoms, preferably 2 to 8, 2 to 6, or 4 to 8 carbon atoms and more preferably 4 or 8 carbon atoms. R<sup>11</sup> is desirably a 2-ethylhexyl group or an n-butyl group.

In one embodiment an aromatic amine antioxidant is used in combination with the additive formulation and the sterically hindered phenol. The aromatic amines can be represented by the formula:



wherein R<sup>12</sup> and R<sup>13</sup> are independently a hydrogen or an arylalkyl group or a linear or branched alkyl group containing 1 to 24 carbon atoms and h is independently 0, 1, 2, or 3, provided that at least one aromatic ring contains an arylalkyl group or a linear or branched alkyl group. Preferably R<sup>12</sup> and R<sup>13</sup> are alkyl groups containing from 4 to 20 carbon atoms. A preferred embodiment is an alkylated diphenylamine such as nonylated diphenylamine of the formula:



#### Dispersants

Dispersants are well known in the field of lubricants and include primarily what are sometimes referred to as "ash-less" dispersants because (prior to mixing in a lubricating composition) they do not contain ash-forming metals and they do not normally contribute any ash forming metals when added to a lubricant. Dispersants are characterised by a polar group attached to a relatively high molecular weight hydrocarbon chain.

One class of dispersant is Mannich bases. These are materials which are formed by the condensation of a higher molecular weight, alkyl substituted phenol, an alkylene polyamine, and an aldehyde such as formaldehyde. Such materials (including a variety of isomers) and are described in more detail in U.S. Pat. No. 3,634,515.

Another class of dispersants is succinimide compounds. These materials are formed by the reaction of a hydrocarbyl substituted succinic acylating agent and an amine. A more detailed description of succinimide compounds suitable for the invention are described in European patent 976 814.

Another class of dispersants is high molecular weight esters. This class of dispersant is described in more detail in U.S. Pat. No. 3,381,022.

Other dispersants include polymeric dispersant additives, which are generally hydrocarbon-based polymers which contain polar functionality to impart dispersancy characteristics to the polymer.

A preferred class of dispersants is the carboxylic dispersants. Carboxylic dispersants include succinic-based dispersants, which are the reaction product of a hydrocarbyl substituted succinic acylating agent with an organic hydroxy compound or, preferably, an amine containing at least one hydrogen attached to a nitrogen atom, or a mixture of said hydroxy compound and amine. The term "succinic acylating agent" refers to a hydrocarbon-substituted succinic acid or succinic acid-producing compound. Such materials typically include hydrocarbyl-substituted succinic acids, anhydrides, esters (including half esters) and halides. Succinimide dispersants are more fully described in U.S. Pat. No. 4,234,435.

#### Antiwear Agents

The lubricant may additionally contain an antiwear agent. Useful antiwear agents include but are not limited to a metal thiophosphate, especially a zinc dialkyldithiophosphate; a

phosphoric acid ester or salt thereof; a phosphite; and a phosphorus-containing carboxylic ester, ether, or amide. A more detailed discussion and examples of phosphorus containing compounds suitable as antiwear agents is discussed in European patent 612 839.

#### Boron Containing Compounds

The lubricant may additionally contain one or more borated compounds. Useful borated compound include borate esters, borated fatty amines, borated epoxides, and borated dispersants such as borated succinimide dispersants, such as are disclosed in U.S. Pat. No. 5,883,057, columns 29-33. Some useful boron-containing compounds may be represented by one or more of the formulas



where each R is independently an organic group and any two adjacent R groups may together form a cyclic group. In one embodiment, R is a hydrocarbyl group. The total number of carbon atoms in the R groups in each formula should be sufficient to render the compound soluble in base oil. Generally, the total number of carbon atoms in the R groups is at least 8 or at least 12. There is no rigid limit to the total number of carbon atoms in the R groups, but a practical upper limit is 400 or 500 carbon atoms. Examples of useful R groups include isopropyl, n-butyl, isobutyl, amyl, 4-methyl-2-pentyl, 2-ethyl-1-hexyl, isoctyl, decyl, dodecyl, tetradecyl, 2-pentenyl, dodecanyl, phenyl, naphthyl, alkylphenyl, alkylnaphthyl, phenylalkyl, naphthylalkyl, alkylphenylalkyl, and alkylnaphthylalkyl.

In certain embodiments, the boron-containing compound can be represented by the formulas B(OC<sub>5</sub>H<sub>11</sub>)<sub>3</sub> or B(OC<sub>4</sub>H<sub>9</sub>)<sub>3</sub> or B(O—CH<sub>2</sub>—CH(C<sub>2</sub>H<sub>5</sub>)—C<sub>4</sub>H<sub>9</sub>)<sub>3</sub>. A useful boron-containing compound is available from Mobil under the trade designation MCP-1286, identified as a borated ester.

The boron-containing compound (B) can be a compound represented by the formula



where: R<sup>1</sup>, R<sup>2</sup>, R<sup>3</sup> and R<sup>4</sup> are independently hydrocarbyl groups of 1 to 12 carbon atoms; and R<sup>5</sup> and R<sup>6</sup> are independently alkylene groups of 1 to 6 carbon atoms, and in one embodiment 2 to 4 carbon atoms. A useful phenolic borate is available from Crompton Corporation under the trade designation LA-2607.

## 15

The boron-containing compound can be a compound represented by the formula:



where: R<sup>1</sup>, R<sup>2</sup>, R<sup>3</sup>, R<sup>4</sup>, R<sup>5</sup>, R<sup>6</sup>, R<sup>7</sup> and R<sup>8</sup> are independently hydrogen or hydrocarbyl groups. Each of the hydrocarbyl groups may contain from 1 to 12 carbon atoms, and in one embodiment 1 to 4 carbon atoms. An example is 2,2-oxybis-(4,4,6-trimethyl-1,3,2-dioxaborinane).

The boron-containing compound may be employed in the lubricating oil composition at a sufficient concentration to provide a boron concentration of 0.01 to 0.2% by weight, or 0.015 to 0.12% by weight, or 0.05 to 0.1% by weight. A discussion and examples of certain alkylated borates is found in European patent 976 814.

## Friction Modifiers

The lubricant may additionally contain a friction modifier. Useful friction modifiers include fatty amines, esters, especially glycerol esters such as glycerol monooleate, borated glycerol esters, fatty phosphites, fatty acid amides, fatty epoxides, borated fatty epoxides, alkoxylated fatty amines, borated alkoxylated fatty amines, metal salts of fatty acids, sulfurized olefins, fatty imidazolines, condensation products of carboxylic acids and polyalkylene-polyamines, amine salts of alkylphosphoric acids, and molybdenum-containing friction modifiers such as molybdenum dithiocarbamates. Among suitable molybdenum friction modifiers are molybdenum and sulfur-containing compositions derived from a molybdenum compound, a basic nitrogen-containing compound, and carbon disulfide. The basic nitrogen compound can be a hydrocarbyl amine or a reaction product of a carboxylic acid with an alkylene polyamine. The molybdenum compound can be an acidic Mo compound such as molybdic acid. An example of such a friction modifier is the reaction product of polyethylenamine bottoms with isostearic acid, further treated with MoO<sub>3</sub> and H<sub>2</sub>O and then carbon disulphide.

## Viscosity Modifiers

The lubricant may additionally contain a viscosity modifier. Viscosity modifiers comprising from polyolefins or polyacrylates are well known in the art.

The lubricating compositions are particularly effective as engine lubricating oils having enhanced antiwear properties. These lubricating compositions are effective in a variety of applications including crankcase lubricating oils for spark-ignited and compression-ignited internal combustion engines, including automobile and truck engines, two-cycle engines, aviation piston engines, marine and low-load diesel engines.

## EXAMPLES

The following examples illustrate the invention. It should however be noted that these examples are non exhaustive and not intended to limit the scope of the invention.

## 16

## Example 1

## Preparation of a Conventional Lubricant Formulation (Comparative)

Hereinafter the term "CLF" is used for the Conventional Lubricant Formulation. A CLF 10 W-30 formulation is prepared containing 95 percent of 200N API Group 3 base oil, 7 mm<sup>2</sup>s<sup>-1</sup> (cSt) at 100° C. and 5 percent of 100N Group 3 base oil, 4 mm<sup>2</sup>s<sup>-1</sup> (cSt) at 100° C. Additionally, 3.5 percent of a viscosity modifier (olefin copolymer) and 0.3 percent pour point depressant are added to the lubricant formulation.

The following additives are added to the 10 W-30base oil formulation (weight percents based on the total lubricant formulation):

|         |                                                        |
|---------|--------------------------------------------------------|
| 7.2%    | Succinimide dispersant(s), 50% chemical in diluent oil |
| 2.1%    | Calcium sulphonate detergent(s), including diluent oil |
| 1.6%    | Calcium phenate detergent(s), including diluent oil    |
| 1.15%   | ZDDP antiwear agent, including diluent oil             |
| 0.50%   | Sulphur-containing antioxidant                         |
| 0.03%   | Copper passivator                                      |
| 0.4%    | Additional diluent oil                                 |
| 100 ppm | Silicone antifoam agent (commercial)                   |

## Example 2

## Preparation of Inventive Lubricant Formulation

Hereinafter the term "ILF" is used for the Inventive Lubricant Formulation. A ILF 10 W-30 formulation is prepared containing 87 percent of 200N API Group 3 base oil, 7 mm<sup>2</sup>s<sup>-1</sup> (cSt) at 100° C. and 13 percent of 100N Group 3 base oil, 4 mm<sup>2</sup>s<sup>-1</sup> (cSt) at 100° C. Additionally, 2.7 percent of a viscosity modifier (olefin copolymer) and 0.3 percent pour point depressant are added to the lubricant formulation.

The following additives are added to the 10 W-30base oil formulation (weight percents based on the total lubricant formulation):

|       |                                                                                                                                                                                  |
|-------|----------------------------------------------------------------------------------------------------------------------------------------------------------------------------------|
| 10.0% | Succinimide dispersant(s), ~60% chemical in diluent oil                                                                                                                          |
| 0.50% | ZDDP antiwear agent, 91% active chemical in diluent oil                                                                                                                          |
| 1.3%  | Borate ester                                                                                                                                                                     |
| 2.1%  | Magnesium saligenin detergent, about 63 TBN, prepared from dodecyl-phenol and paraformaldehyde (as prepared in U.S. Pat. No. 6,310,009, Example 1), 50% chemical in diluent oil. |
| 1.9%  | 150 TBN Calcium Salixarate (as prepared in preparative example A), 65% chemical in diluent oil                                                                                   |
| 0.6%  | 400 TBN Overbased calcium alkylbenzene sulphonate detergent, 58% chemical in diluent oil                                                                                         |
| 4%    | Hindered phenolic ester antioxidant                                                                                                                                              |
| 1.5%  | Aromatic amine antioxidant                                                                                                                                                       |
| 0.6%  | Sulphur-containing antioxidant                                                                                                                                                   |
| 0.01% | Silicone defoamer (commercial material containing about 90% diluent)                                                                                                             |

Samples of the formulations described above are evaluated for their performance in wear, oxidation, seal compatibility, elemental analysis, ash content and deposit tests.

## Test 1

Elemental analysis studies are carried out on CLF and ILF samples. The results obtained are presented in Table 1.

TABLE 1

| Elemental Analysis |            |            |
|--------------------|------------|------------|
| Element            | CLF (wt %) | ILF (wt %) |
| B                  |            | 0.0524     |
| Ca                 | 0.2759     | 0.1804     |
| Mg                 |            | 0.0317     |
| P                  | 0.1147     | 0.0492     |
| S                  | 0.4090     | 0.1977     |
| Si                 | <0.001     | <0.001     |
| Zn                 | 0.1280     | 0.0563     |

The analysis indicates ILF contains significantly less sulphur, phosphorus, zinc and calcium.

#### Test 2

The amount of deposition is established using the Panel Coker Deposit Test. In this test, the sample, at 105° C., is splashed for 4 hours on an aluminium panel maintained at 325° C. The aluminium plates are analysed using image analysis techniques to obtain a universal rating. The rating score is based on 100 being a clean plate and 0 a plate wholly covered in deposit. The universal ratings obtained for CLF and ILF samples are 28 and 86 respectively. The higher universal rating for the ILF sample indicates significant improvements over the CLF sample.

#### Test 3

The amount of viscosity increase caused by lubricant oxidation in marine trunk piston engine oils is established, by measuring the viscosity at 40° C. before and after heating the oil to 200° C. and holding for 24 hours. Air is blown into the system at a 25 cc min<sup>-1</sup>. Lower percentage viscosity increases indicate better performance. The results obtained for CLF and ILF samples are:

|                               | CLF     | ILF   |
|-------------------------------|---------|-------|
| 0 hours viscosity at 40° C.   | 69.57   | 74.08 |
| 24 hours viscosity at 40° C.  | 109.247 | 99.24 |
| Percentage viscosity increase | 57      | 34    |

The analysis indicates lubricating oils with ILF have viscosity increases significantly less than those with CLF.

#### Test 4

Seal compatibility tests are designed to evaluate the effect of motor oils on Parker-Pradifa™ FKM E-281 seal elastomers (fluoroelastomer). Six dumb-bells of elastomer are suspended using a micro wire and glass separators are covered by at least 10 ml of oil. The test vessel is covered with aluminium foil and stored at 150° C. for 96 hours. The elastomer is removed from the oil and tested for percentage change in tensile strength, elongation, and cracking (by bending). The results obtained for CLF and ILF samples are:

|                   | CLF     | ILF         |
|-------------------|---------|-------------|
| tensile change    | -47.2   | -18.9       |
| elongation change | -43.3   | -24.4       |
| bend test         | cracked | not cracked |

The analysis indicates lubricating oils with ILF have improved seal compatibility over those with CLF, that is,

#### 18

compared with a control formulation with the combination of calcium sulphonate and calcium phenate detergents, without the saligenin and salixarate detergents.

#### Test 5

Nitration experiments are carried out on 40 gram oil samples by mixing 0.17 ml of 6N nitric acid and 0.09 ml of 0.5% iron naphthenate into the oil and heating to 145° C. for 22 hours. NO<sub>x</sub> is blown into the system at a rate of 25 cc min<sup>-1</sup>. The sample of oil is removed and analysed for changes in the FTIR profile for RONO<sub>2</sub>, a characteristic nitration functionality, by appearance of the corresponding peak in the IR Samples with small changes in FTIR peak profile (peak height) for RONO<sub>2</sub> are nitrated least. The results obtained for CLF and ILF samples are:

|                   | CLF | ILF |
|-------------------|-----|-----|
| RONO <sub>2</sub> | 9.5 | 7.3 |

The analysis indicates lubricating oils with ILF are less susceptible to nitration than are oils with CLF.

#### Test 6

A High Temperature Cummins Bench Test (HTCBT) is carried out on lubricants to determine their tendency to corrode various metals, specifically lead and copper. Four metal samples of copper, lead, tin and phosphor bronze are immersed in 100 ml of oil and heated to 135° C. for 168 hours with 5 litres of air per hour purging the sample. The ppm levels of copper and lead in the oil are determined at the end of the test. The results obtained for CLF and ILF samples are:

|              | HTCBT Test Data | CLF | ILF |
|--------------|-----------------|-----|-----|
| Copper (ppm) |                 | 10  | 6   |
| Lead (ppm)   |                 | 41  | 2   |

The analysis indicates lubricating oils with ILF have improved resistance to corroding copper and lead over oil with CLF.

#### Test 7

Pressure Differential Scanning Calorimetry (PDSC) is used to determine the ability of oil to resist oxidation. 3 mg of sample is placed in an aluminium pan and isothermally heated to 210° C. and pressurised with oxygen to 3.5 MPa (500 PSIG). The results obtained for CLF and ILF samples are:

|                      | PDSC Oxidation Test | CLF  | ILF   |
|----------------------|---------------------|------|-------|
| Onset time (minutes) |                     | 25.4 | 108.8 |

The analysis indicates lubricating oils with ILF have improved resistance to oxidation over those with CLF.

The results presented in tests 1-7 illustrate the significant reduction in ash, sulphur, and phosphorus in the engine oils of the present invention. The inventive additive formulation produces improved antioxidant, seal compatibility, and cleanliness over conventional formulations.

## Preparation of a Low Emission Formulation with a Conventional Detergent System (Comparative)

Hereinafter the term "LEF CDS" is used for the Low Emission Formulation using the Conventional Detergent System. A LEF CDS 10 W-30 formulation is prepared containing 87 percent of 200N API Group 3 base oil, 7  $\text{mm s}^{-1}$  (cSt) at 100° C. and 13 percent of 100N Group 3 base oil, 4  $\text{mm s}^{-1}$  (cSt) at 100° C. Additionally, 2.7 percent of a viscosity modifier (olefin copolymer) and 0.3 percent pour point depressant are added to the lubricant formulation.

The following additives are added to the 10 W-30 base oil formulation (weight percents based on the total lubricant formulation):

|       |                                                                      |
|-------|----------------------------------------------------------------------|
| 10.0% | Succinimide dispersant(s), ~60% chemical in diluent oil              |
| 0.50% | ZDDP antiwear agent (91% active chemical in diluent oil)             |
| 1.3%  | Borate ester                                                         |
| 1.6%  | Calcium sulphonate detergent(s) including diluent oil                |
| 1.6%  | Calcium phenate detergent(s) including diluent oil                   |
| 4%    | Hindered phenolic ester antioxidant                                  |
| 0.01% | Silicone defoamer (commercial material containing about 90% diluent) |

## Example 4

## Preparation of a Low Emission Formulation with the Inventive Detergent System

Hereinafter the term "LEF IDS" is used for the Low Emission Formulation using the Inventive Detergent System. A LEF IDS 10 W-30 formulation is prepared identical to the material of Example 3, except that the 0.9% calcium sulphonate detergent, the 0.73% overbased calcium sulphonate detergent, the 0.76% calcium phenate detergent, and the 0.87% overbased calcium phenate detergent, are replaced by the following detergent mixture:

2.1% Magnesium saligenin detergent, about 63 TBN, prepared from dodecylphenol and paraformaldehyde (as prepared in U.S. Pat. No. 6,310,009, Example 1), 50% chemical in diluent oil.

1.9% 150 TBN Calcium salixarate as prepared in Preparative Example A, 65% chemical in diluent oil

0.6% 400 TBN Overbased calcium alkylbenzene sulphonate detergent, 58% chemical in diluent oil

Samples of the formulations described above are evaluated for their performance in wear, oxidation, seal compatibility, elemental analysis, ash content and deposit tests.

## Test 1

Elemental analysis studies are carried out on LEF CDS and LEF IDS samples. The results obtained are presented in Table 1.

TABLE 1

| Element | Elemental Analysis |                |
|---------|--------------------|----------------|
|         | LEF CDS (wt %)     | LEF IDS (wt %) |
| B       | 0.0537             | 0.0542         |
| Ca      | 0.2265             | 0.1830         |

TABLE 1-continued

| Element | Elemental Analysis |                |
|---------|--------------------|----------------|
|         | LEF CDS (wt %)     | LEF IDS (wt %) |
| Mg      | 0.0000             | 0.0330         |
| P       | 0.0528             | 0.0518         |
| S       | 0.2263             | 0.1254         |
| Si      | <0.001             | 0.0015         |
| Zn      | 0.0593             | 0.0583         |

## Test 2

The amount of deposition is established using the Panel Coker Deposit Test as described above. The universal ratings obtained for LEF CDS and LEF IDS samples are 14 and 37 respectively. The higher universal rating for the LEF IDS sample indicates significant improvements over the LEF CDS sample.

## Test 3

The amount of viscosity increase caused by lubricant oxidation in marine trunk piston engine oils is established as described above. The results obtained for LEF CDS and LEF IDS samples are:

|                               | LEF CDS | LEF IDS |
|-------------------------------|---------|---------|
| 0 hours viscosity at 40° C.   | 70.69   | 73.48   |
| 24 hours viscosity at 40° C.  | 81.38   | 88.67   |
| Percentage viscosity increase | 15.1    | 20.7    |

The analysis indicates LEF's with IDS have viscosity increases comparable to those with CDS.

## Test 4

Seal compatibility tests are conducted to evaluate the effect of motor oils on Parker-Pradifa™ FKM E-281 seal elastomers (fluoroelastomer) as described above. The results obtained for LEF CDS and LEF IDS samples are:

|                   | LEF CDS | LEF IDS     |
|-------------------|---------|-------------|
| tensile change    | -47.6   | -5.2        |
| elongation change | -36.4   | -20.2       |
| bend test         | cracked | not cracked |

The analysis indicates LEF's with IDS have improved seal compatibility over those with CDS.

## Test 5

Nitration experiments are carried out as described above. The results obtained for LEF CDS and LEF IDS samples are:

|                   | LEF CDS | LEF IDS |
|-------------------|---------|---------|
| RONO <sub>2</sub> | 12.9    | 11.1    |

The analysis indicates LEF's with IDS are comparable or superior in susceptibility to nitration to those with CDS.

## Test 6

A High Temperature Cummins Bench Test (HTCBT) is carried out as described above. The results obtained for LEF CDS and LEF IDS samples are:

| HTCBT Test Data | LEF CDS | LEF IDS |
|-----------------|---------|---------|
| Copper (ppm)    | 4       | 2       |
| Lead (ppm)      | 4       | 1       |

The analysis indicates LEF's with IDS have comparable resistance to corroding copper and lead to oil with CDS.

## Test 7

Pressure Differential Scanning Calorimetry (PDSC) is used to determine the ability of the samples to resist oxidation, as described above. The results obtained for LEF CDS and LEF IDS samples are:

| PDSC Oxidation Test  | LEF CDS | LEF IDS |
|----------------------|---------|---------|
| Onset time (minutes) | 48.8    | 74.9    |

The analysis indicates LEF's with IDS have improved resistance to oxidation over those with CDS.

## Examples 5 and 6

The following formulations are prepared and are subjected to the API CH-4 Cummins M11 Engine test. This test uses a Cummins™ 370-E block engine, which is an electronically governed in-line 6-cylinder 4-stroke, compression ignition engine. The test is conducted in four 50-hour stages. During the first and third stages, the engine is over-fueled and operated with retarded timing to generate soot at an accelerated rate. During the second and fourth stages the engine is run at lower speed and higher torque, to induce wear. The crosshead wear, considered to be representative of valve train wear, is determined and averaged for 12 cross-heads. A passing criterion is considered to be an average weight loss of 6.5 mg or less.

In examples 5 and 6, the amounts of salixarate detergent (Ex. 6) and salicylate detergent (Ex. 5, comparative) are selected to deliver equal amounts of metal, expressed as sulphated ash, the salicylate being a more highly overbased material.

| Component<br>(parts by weight)                                                    | Ex. 5<br>(comparative) | Ex. 6 |
|-----------------------------------------------------------------------------------|------------------------|-------|
| Mixture of 100 N and 200 N API Group III oils                                     | 100                    | 100   |
| Viscosity modifier (including diluent oil)                                        | 2.7                    | 2.7   |
| Pour point depressant (including diluent oil)                                     | 0.3                    | 0.3   |
| 63 TBN Overbased Mg saligenin detergent as described in Ex. 2 (including 50% oil) | 2.1                    | 2.1   |
| 400 TBN Overbased Ca sulphonate detergent (42% oil)                               | 0.6                    | 0.6   |
| 150 TBN Overbased Ca salixarate detergent of Ex. A (35% oil)                      |                        | 1.9   |
| 280 TBN Overbased Ca salicylate detergent (45% oil)                               | 0.95                   |       |

-continued

| Component<br>(parts by weight)                                                                                          | Ex. 5<br>(comparative) | Ex. 6 |
|-------------------------------------------------------------------------------------------------------------------------|------------------------|-------|
| Succinimide dispersants (average 39% oil)                                                                               | 10                     | 10    |
| ZDDP (9% oil)                                                                                                           | 0.5                    | 0.5   |
| Phenolic antioxidant                                                                                                    | 4                      | 4     |
| Dioxylborane (structure B-II-1 where R <sup>1</sup> and R <sup>3</sup> are H and the remaining Rs are CH <sub>3</sub> ) | 0.75                   | 0.75  |
| 10 Antifoam agent (commercial)                                                                                          | 0.01                   | 0.01  |
| M11 Average Crosshead Wear (mg)                                                                                         | 10.6                   | 5.7   |

## Example 7

15 Example 6 is repeated except that the dioxylborane is replaced by 1.3 parts n-butyl borate ester.

## Examples 8 and 9

20 Example 7 is repeated except that the detergent component (saligenin, sulphonate, and salixarate, above) is replaced by the following detergent components, in parts by weight:

| Detergent component (parts by weight)                                             | Ex. 8 | Ex. 9 |
|-----------------------------------------------------------------------------------|-------|-------|
| 63 TBN Overbased Mg saligenin detergent as described in Ex. 2 (including 50% oil) | 1.05  | 1.05  |
| 30 400 TBN Overbased Ca sulphonate detergent (42% oil)                            | 0.45  | 0.45  |
| 150 TBN Overbased Ca salixarate detergent of Ex. A (35% oil)                      | 1.3   | 1.3   |
| 255 TBN Overbased Ca dodecyl phenate sulphide detergent (39% oil)                 | 0.75  | —     |
| 35 165 TBN Overbased Ca alkyl salicylate detergent (40% oil)                      | —     | 1.15  |

While the invention has been explained in relation to its preferred embodiments, it is to be understood that various 40 modifications thereof will become apparent to those skilled in the art upon reading the specification. Therefore, it is to be understood that the invention disclosed herein is intended to cover such modifications as fall within the scope of the appended claims.

45 Each of the documents referred to above is incorporated herein by reference. Except in the Examples, or where otherwise explicitly indicated, all numerical quantities in this description specifying amounts of materials, reaction conditions, molecular weights, number of carbon atoms, and 50 the like are to be understood as modified by the word "about." Unless otherwise indicated, each chemical or composition referred to herein should be interpreted as being a commercial grade material which may contain the isomers, by-products, derivatives, and other such materials which are 55 normally understood to be present in the commercial grade.

However, the amount of each chemical component is presented exclusive of any solvent or diluent oil, which may be customarily present in the commercial material, unless otherwise indicated. It is to be understood that the upper and 60 lower amount, range, and ratio limits set forth herein may be independently combined. Similarly, the ranges and amounts for each element of the invention can be used together with ranges or amounts for any of the other elements. As used herein, the expression "consisting essentially of" permits the 65 inclusion of substances that do not materially affect the basic and novel characteristics of the composition under consideration.

What is claimed is:

1. A method of lubricating a compression-ignited internal combustion engine, comprising supplying thereto a lubricant composition comprising:
  - (a) about 0.05 to about 1.5 weight percent of a calcium or magnesium sulphonate detergent;
  - (b) about 0.2 to about 2 weight percent of a calcium salixarate detergent;
  - (c) about 0.2 to about 1.7 weight percent of a magnesium saligenin detergent; and
  - (d) an oil of lubricating viscosity in an amount up to about 99.75 weight percent, wherein the composition has a total sulphur content of below about 0.5 weight percent and a total phosphorus content of below about 0.1 weight percent.

2. The method according to claim 1, wherein said saligenin detergent is represented by the formula:



wherein, X comprises  $-\text{CHO}$  or  $-\text{CH}_2\text{OH}$ , Y comprises  $-\text{CH}_2-$  or  $-\text{CH}_2\text{OCH}_2-$ , and wherein such  $-\text{CHO}$  groups comprise at least about 10 mole percent of the X and Y groups; M is a calcium, magnesium, lithium, potassium or sodium ion; each n is independently 0 or 1;  $R^1$  is a hydrocarbyl group containing 1 to about 60 carbon atoms; m is 0 to about 10, and when  $m > 0$ , one of the X groups can be H; each p is independently 0, 1, 2 or 3; and the total number of carbon atoms in all  $R^1$  groups is at least 7.

3. The method according to claim 1, wherein said salixarate detergent is represented by a substantially linear compound comprising at least one unit of formula (I) or formula (II):



each end of the compound having a terminal group of formula (III) or formula (IV):



20 such groups being linked by divalent bridging groups A, which may be the same or different for each linkage; wherein in formula (I)-(IV) it  $R^3$  is hydrogen or a hydrocarbyl group;  $R^2$  is hydroxyl or a hydrocarbyl group and j is 0, 1, or 2;  $R^6$  is hydrogen, a hydrocarbyl group, or a hetero-substituted hydrocarbyl group; either  $R^4$  is hydroxyl and  $R^5$  and  $R^7$  are independently either hydrogen, a hydrocarbyl group, or hetero-substituted hydrocarbyl group, or else  $R^5$  and  $R^7$  are both hydroxyl and  $R^4$  is hydrogen, a hydrocarbyl group, or a hetero-substituted hydrocarbyl group; provided that at least one of  $R^4$ ,  $R^5$ ,  $R^6$  and  $R^7$  is hydrocarbyl containing at least 8 carbon atoms; and wherein the molecules on average contain at least one of unit (I) or (III) and at least one of unit (II) or (IV) and the ratio of the total number of units (I) and (III) to the total number of units of (II) and (IV) in the method is about 0.1:1 to about 2:1.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930

**25**

11. The method of claim **1** further comprising a friction modifier.

12. The method of claim **11** wherein the friction modifier is a molybdenum compound.

13. The method of claim **1** further comprising a borate ester or a borated succinimide dispersant.

14. The method of claim **1** further comprising an antiwear agent.

**26**

15. The method of claim **14** wherein the antiwear agent comprises a zinc dialkyl dithiophosphate.

16. The method of claim **1** further comprising a dispersant.

17. The method of claim **1** wherein the oil of lubricating viscosity comprises an API Group II, Group III, Group IV, or Group IV oil or mixtures thereof.

\* \* \* \* \*